

No. 843,683.

PATENTED FEB. 12, 1907.

H. MANNHARDT,  
METAL AND CONCRETE STRUCTURE,  
APPLICATION FILED NOV. 7, 1906.



Witnesses:

Andrew Summer  
L. A. Smith

Inventor,  
Hans Mannhardt  
by Summer & Summer,  
Attorneys.

# UNITED STATES PATENT OFFICE.

HANS MANNHARDT, OF CHICAGO, ILLINOIS.

## METAL AND CONCRETE STRUCTURE.

No. 843,683.

Specification of Letters Patent.

Patented Feb. 12, 1907.

Application filed November 7, 1906. Serial No. 342,378.

*To all whom it may concern:*

Be it known that I, HANS MANNHARDT, a citizen of the United States of America, and a resident of Chicago, in the county of Cook and State of Illinois, have invented certain new and useful Improvements in Metal and Concrete Structures, of which the following is a specification.

The objects of this invention are to provide an improved building structure in which iron or other corrosive metal is surrounded by or covered with concrete and to effectively prevent the corrosion of the metal; also, to provide for coating the metal with a protective non-corrosive non-hygrosopic film after the metal structure has been erected, as in a building, and before the concrete is built up around the same. These objects are accomplished by the structure illustrated in the accompanying drawing and hereinafter described.

The drawing shows a cross-section of a pillar formed of a channel-bar 1, surrounded by concrete 2 and having an intervening protective film 3. Heretofore in building structures consisting of corrosive metal surrounded by concrete the metal has usually been coated with a varnish or paint containing a drying-oil and the concrete has then been built up around this film. The drying-oil used in the film causes the film to become spongy and permeable to moisture through the action of the gases liberated in the oxidation. This has resulted in the corrosion and comparatively rapid deterioration of the metal. Such corrosion can be prevented by avoiding the use of drying-oils and using as a coating for forming the protective film some volatile solvent—such as benzene, benzole, turpentine, carbon disulfid, carbon tetrachlorid, chloroform, methyl or ethyl alcohol—in which is held in solution a suitable body formed of resins, metallic resinate, vegetable, animal, or mineral oils, (excepting drying-oils,) and fats or waxes or similar materials.

The main feature of the material from which the coating or film used in this invention is formed is that it is adhesive and will flow readily, so as to be readily painted or

spread upon the metallic structure after the same has been erected in a building construction or that it will form a uniform coating upon the metallic structure when the latter is dipped therein and which shall be free from all drying-oils, so that when the solvent in said coating has volatilized the remaining film will be non-corrosive, non-corrodible, non-permeable to moisture and gases, and non-hygrosopic. Such film may be made by taking a solution containing one part, by weight, of resinate of lime to nine parts, by weight, of benzene and mixing the same, usually at ordinary temperature, and then brushing or spraying the solution upon the metal structure and permitting it to dry thereon before the concrete is built up around the same. When practicable, the metal structure may be dipped in a similar solution. In either case when the solution dries a film is formed having the characteristics above mentioned. An advantage of using resinate of lime in such solution is that the concrete, which contains lime, will not form a disintegrating chemical combination, which might be formed if some other substances are used instead of the resinate of lime as a body for the film.

What I claim as my invention, and desire to secure by Letters Patent, is—

1. A metal core having its surface coated with a non-corrosive, non-hygrosopic film formed by the evaporation of a volatile solvent carrying in solution a non-corrosive, non-hygrosopic adhesive body, free from drying-oil, and having a concrete covering in contact with said film.

2: A metal core having its surface coated with a film formed by the evaporation of a volatile solvent carrying in solution a resinate of lime, being free from drying-oil, and having a concrete covering in contact with said film.

Signed at Chicago this 3d day of November, 1906.

HANS MANNHARDT:

Witnesses:

RUDOW RUMMLER,  
W.M. R. RUMMLER